

## 1

3,536,438

### PROCESS OF DYEING TEXTILE FIBRES USING A PHENYL SULPHONE DYEING ASSISTANT

Hans-Peter Baumann, Munchenstein, and Robert-Christian Keller, Basel, Switzerland, assignors to Sandoz Ltd., Basel, Switzerland, a corporation of Switzerland  
No Drawing. Filed Mar. 3, 1967, Ser. No. 620,232  
Claims priority, application Switzerland, Mar. 11, 1966,

3,576/66

Int. Cl. D06p 3/82

U.S. Cl. 8—21

14 Claims

#### ABSTRACT OF THE DISCLOSURE

Dyeing process for nylon and mixed nylon/urethane fibres, yarn and fabrics with anionic dyestuffs using dyeing assistants to prevent stripy or ringy dyeings and/or uneven dye adsorption on the nylon and on the urethane fibres. The dyeing assistants exemplified are sulphonated sulphones derived from hydroxybenzene, 1-hydroxy-4-phenylbenzene, 1-hydroxy-3-methylbenzene, 1-hydroxy-2-chlorobenzene, methoxybenzene, dibenzofuran, 3-hydroxy-diphenylene oxide, methylbenzene, diphenyl oxide, phenoxy-diphenyl, diphenyl sulphide, water soluble salts of these phenyl sulphones and water soluble reaction products of them with formaldehyde or dimethylol urea.

#### BACKGROUND OF THE INVENTION

Polyamide fibres can be dyed with anionic dyestuffs, but frequently the resulting dyed goods have a stripy or ringy appearance due to an uneven adsorption and distribution of dye. Furthermore, mixtures of polyamide fibres and elastomeric polyurethane fibres or yarns as are used for making woven or knitted fabrics cannot easily be level dyed in equal colour shades with anionic dyestuffs as these are preferentially adsorbed on the polyamide fibres, thus leaving the polyurethane fibres in a much paler shade and causing the fabrics to be stripy.

It has previously been proposed to use certain levelling agents to minimize the above difficulties, but these previously proposed levelling agents have not been entirely satisfactory for use or more of the following reasons: insufficient penetration power, necessity to effect a relatively troublesome separate treatment before dyeing, relatively high price of the levelling agent, and difficulties in handling these due to their being non-solids at ambient temperature.

We have now found that the use of certain sulphonated phenyl sulphones described hereinafter and which have an excellent penetration power enables one to dispense with a separate pretreatment before dyeing and to use relatively inexpensive products which, moreover, can be handled very easily because they are obtainable in the solid state at room temperature.

#### SUMMARY OF THE INVENTION

The present invention provides a process for dyeing with anionic dyestuffs textile fibres of polycondensation products containing carbonamide groups, which have varying affinity to anionic dyestuffs, characterized in that the fibres are treated with an aqueous solution of a phenyl sulphone optionally substituted and containing at least one  $-\text{SO}_3-$  (cation) radical attached to an aromatic nucleus and at least one radical of the formula

R—X—

wherein X represents  $-\text{O}-$  or  $-\text{S}-$  and R represents a hydrogen atom or low molecular weight alkyl radical optionally substituted, a phenyl-, phenylalkyl- or diphenyl radical optionally substituted or an ortho-phenyl-

## 2

radical optionally substituted which forms a furan or thiophene ring with the benzene ring adjacent to X, or of a condensation product thereof with formaldehyde or a nitrogen containing polyfunctional connecting agent containing at least one methylol radical.

#### DETAILED DESCRIPTION

Examples of suitable cations, due to whose presence the sulphonated phenyl sulphones are rendered water soluble, are  $\text{H}^+$  alkali metal ions, preferably  $\text{Na}^+$  and  $\text{K}^+$ , further  $\text{Mg}^{++}$ ,  $\text{Ca}^{++}$ ,  $\text{NH}_4^+$  and amines, for instance  $\text{CH}_3-\text{NH}_3^+$ ,  $(\text{CH}_3)_2\text{NH}_2^+$ ,  $(\text{CH}_3)_3\text{NH}^+$ ,  $\text{C}_2\text{H}_5-\text{NH}_3^+$ ,  $\text{HO}-\text{C}_2\text{H}_4-\text{NH}_3^+$ ,  $(\text{HO}-\text{C}_2\text{H}_4)_2-\text{NH}_2^+$ ,  $(\text{HO}-\text{C}_2\text{H}_4)_3\text{NH}^+$

15 and others more.

The radical R—X— in the phenyl sulphones is preferably an R—O— radical, wherein R has the above significance, and especially an  $\text{R}_1-\text{O}-$  radical, wherein  $\text{R}_1$  is a hydrogen atom or a low molecular weight alkyl radical which may be substituted, or an optionally substituted phenyl-, phenylalkyl- or diphenyl radical; examples of  $-\text{O}-\text{R}_1$  are therefore  $-\text{OH}$ ,  $-\text{O}-\text{CH}_3$ ,  $-\text{O}-\text{C}_2\text{H}_5$ ,  $-\text{O}-\text{phenyl}$ ,  $-\text{O}-\text{benzyl}$ ,  $-\text{O}-\text{diphenyl}$ ,



wherein n is from 1 to 3, further



wherein "alkyl" contains 2 to 5 carbon atoms, or



40 The preferred meaning of  $-\text{O}-\text{R}_1$ , however, is  $-\text{OH}$ ,  $-\text{O}-\text{phenyl}$  or  $-\text{O}-\text{diphenyl}$ .

45 The sulphonated phenyl sulphones used in the dyeing process of the invention are agents which are capable of regulating the speed of adsorption and distribution of anionic dyestuffs on the fibres to be dyed.

50 By "anionic dyestuffs" are designated dyestuffs which are capable of forming coloured anions in aqueous dye liquor, for example acid level dyestuffs, fulling dyestuffs, 1:1- and 1:2-metal complex dyestuffs, chrome dyes, direct dyes and reactive dyes.

55 Textile fibres of polycondensation products containing carbonamide radicals and having varying affinity to anionic dyestuffs include synthetic polyamide fibres or polyurethane fibres becoming stripy or ringy on dyeing and mixtures of these fibres. Examples of polyamide fibres are nylon 6, 66, 610 6/66, 11, etc.; examples of polyurethane fibres are polycondensation products of diols and diisocyanates, e.g., of 1,4-butane diol and 1,6-hexamethylene-diisocyanate, or mixed condensation products of polyethers or polyesters with diisocyanates and diamines or hydrazine [Ullmann Enzyklopädie der technischen Chemie 14, 338,363, especially 351-2 (1963)].

60 The new dyeing process is especially suitable for dyeing mixtures of synthetic polyamide fibres and elastomeric fibres of polyurethanes. Such mixtures have become increasingly more important in the last few years. Taken individually, both kinds of fibres are capable of being dyed with anionic dyestuffs. However, simultaneous dyeing of polyamide and elastomeric fibres with anionic dyestuffs entails difficulties, as the dyestuffs are not built up in the same way on both kinds of fibres. Mostly the polyamide fibre part becomes dyed quicker and in a deeper shade than the elastomeric fibre portion. It is therefore

not easily possible to achieve an equal shade or level tint on dyeing these two kinds of fibres simultaneously, for example a dyeing in a uniform shade, or to obtain a darker shade with the elastomeric fibres than with the polyamide fibres.

Elastomeric or spandex fibres have a high elasticity and the fibre forming substance is a chain-like polymer which mainly consists of segmented polyurethane. These fibres are produced and sold commercially under various trade names [for these trade names see, e.g., H. U. Schmidlin, SVF-Fachorgan 20, (1965) No. 2, page 8].

Threads or yarns containing a portion of spandex fibres are commercially available, for example, under the name of corespun yarns in the production of which endless elastomeric threads are wrapped round with polyamide staple yarns; alternatively they are available as staple fibres which are obtained by spinning polyamide staple fibres with cut elastomeric threads.

Suitable synthetic polyamide fibres which may be dyed together with elastomeric fibres include the most varied fibres consisting of synthetic polyamide and also such as are subjected to a special treatment, e.g. texturizing. Such products are known, for example, under the following names some of which are registered: nylon 6, nylon 6,6, nylon 66/6, nylon 10, "Grilon," "Perlon," "Mirlon," "Enkalon," "Tastan," "Stylon," "Rilsan," "Ban-lon," "Dederon," etc.

The fibres or fibre mixtures to be dyed in accordance with the process of the invention, preferably those of elastomer and polyamide fibres, may take any desired form, for example free fibres, threads, woven or knitted fabrics, or made up goods, e.g. pullovers, articles of fashion, shirts and sports clothing.

The optionally substituted phenyl sulphones to be used in accordance with the invention and containing at least one aromatically linked  $-\text{SO}_3-$  (cation)-radical and at least one radical of the formula  $\text{R}-\text{X}-$ , wherein R and X have the above significance, may be obtained in accordance with known methods. Suitable one uses as starting material a compound of the formula



wherein A is a phenyl radical optionally substituted with one or more halogen atoms, hydroxy radicals, alkyl radicals containing 1-4 carbon atoms, or a diphenyl radical, and X and R have the above significance, or a mixture of two or more such compounds and converts to the corresponding monosulphonic acid. Conversion of the last mentioned to the corresponding phenyl sulphone containing sulphonic acid radicals may be effected, for example, by heating to 100-200° C. at a reduced pressure; the resulting product is soluble in water in the form of the alkali metal salt. The phenyl sulphone, depending on the nature of the starting material and the reaction conditions, contains one or more  $-\text{SO}_2-$  radicals per molecule. In general, the phenyl sulphones to be used in accordance with the invention are mixtures of mono- and poly-(phenyl sulphones), e.g. of mono-, di-, tri-, tetra-, and penta-(phenyl sulphones), the average  $-\text{SO}_2-$  radical content per molecule being preferably 1 to 3. Furthermore, other products usable in accordance with the invention are obtained when the resulting phenyl sulphones are additionally reacted with formaldehyde or with connecting agents containing methylol radicals, for example dimethylol urea.

Suitable compounds of the formula



are, for example, phenol, 2-chlorophenol, 4-phenylphenol, 3-methylphenol, anisole, phenetole, diphenyl oxide, phenoxy diphenyl, diphenylsulphide, dibenzofuran and 3-hydroxydibenzofuran. The production of phenyl sulphones to be used in accordance with the invention is described, e.g., in German patent specifications Nos. 260,379; 265,415; 266,124; 266,139; 825,090 and 819,694. The conditions of dyeing are substantially those usual for the dif-

ferent types of anionic dyestuffs, e.g. temperatures of from 80° to 140° C., preferably 95° to 130° C., and at super atmospheric pressure when the dyeing temperature exceeds 100° C.; bath liquor ratios of from 1:5 to 1:200, preferably of 1:10 to 1:100; pH values of 2 to 8, depending on the dyeing properties of the dyestuffs used when the treatment of the fibres with the sulphonated phenyl sulphones is effected in the dye bath itself. However, the treatment with the sulphonated phenyl sulphones may be effected before the actual dyeing at temperatures of about 20° C. to 100° C., preferably at 50° to 100° C. and in slightly acid medium, e.g. acetic acid medium.

The fibres treated in this way may be removed from the treatment liquor, rinsed with water, if desired dried and then put in a freshly prepared dye bath and dyed therein, or may be dyed after treatment in the same liquor after the addition of a dyestuff and any dyeing assistants (salts, acids, metallizing agents, surface active agents, etc.).

The amount of sulphonated phenyl sulphone to be used in accordance with the process depends on the nature of the fibres to be dyed, on the quantity and structure of the dyestuff used for dyeing, the pH value of the dyeing liquor, the dyeing temperature and the duration of the obtained. It amounts to from 0.02 to 20% by weight, preferably 0.1 to 15% by weight, of the material to be dyed. In addition to the sulphonated phenyl sulphone to be used in accordance with the process of the invention, it is possible to add to the dye baths one or more buffer substances, e.g. hexamethylenetetramine, disodium phosphate, tetrasodium pyrophosphate, urea or ammonium rhodanide. If desired it is possible to use for dyeing also one or more non-ionogenic, anionic or cationic, capillary active compounds, providing this does not lead to the formation of a precipitate with the dyestuff and the sulphonated phenyl sulphone. The dyeing of, e.g. spandex/nylon mixtures is advantageously effected in such a way that the phenyl sulphone to be used in accordance with the process of the invention is either added to the dye bath together with the dyestuff and dyeing is effected as usual, or the mixed material is first pretreated with a solution of the sulphonated phenyl sulphone, the dyestuff is then added and dyeing effected. However, it is likewise possible to proceed in such a way that the fibres, e.g. a mixture of elastomeric and synthetic polyamide fibres, are first subjected to a pretreatment with a solution of the sulphonated phenyl sulphone, the dyestuff is then added and dyeing effected. However, it is likewise possible to proceed in such a way that the fibres, e.g. a mixture of elastomeric and synthetic polyamide fibres, are first subjected to a pretreatment with a solution of the sulphonated phenyl sulphone and then dyed without intermediate drying in a freshly prepared dye bath.

The dyeing process in accordance with the invention can, however, likewise be effected in such a way that the synthetic polyamide is subjected to treatment with the sulphonated phenyl sulphone to be used in accordance with the process of the invention before processing to give a fibre mixture of elastomer-polyamide.

The sulphonated phenyl sulphone to be used in accordance with the process of the invention may be prepared, for example, in the following manner; the sulphones are mixtures constituted by monomers and polymers essentially having up to 5 recurring units,  $n'$  thus being 0, 1, 2, 3 or 4 and Ph being the phenyl or phenylene radical respectively,  $n=1, 2$  or 3 and  $m=1$  or 2.

#### PHENYL SULPHONE A

102 parts of 100% sulphuric acid (1.04 mols) are slowly added to 94 parts of hydroxybenzene (1 mol) and heated for 4 hours to 100° C. Subsequently the pressure is reduced to 20 mm. of Hg, the temperature is increased during 2 hours to 160° C. and condensation is effected for 4 hours at 160° C. The pressure is then further reduced to 3 mm. of Hg and the temperature is simultaneously increased to 180° C. Condensation is then



and the temperature increased to 150° C. Condensation is then effected until a sample of the condensate has an acid content of 350 mval./100 g. of resin (titrated against Congo red).

The sulphone has the following formula:



#### PHENYL SULPHONE M

Working is effected as for the production of the phenyl sulphone K, but using 127.5 parts of diphenyl oxide and 70.5 parts of hydroxy benzene and the condensation is effected at 160° C. and 3 mm. of Hg until the acid content has fallen to 355 mval./100 g. of product (titrated against Congo red).

#### PHENYL SULPHONE N

Working is effected as for the production of phenyl sulphone K, but using 186 parts of diphenyl sulphide. The resulting product has an acid content of 375 mval./100 g. (titrated against Congo red). The product has the formula:



#### PHENYL SULPHONE O

50 parts of the phenyl sulphone A are mixed with 10 parts of water and 23 parts of 30% sodium hydroxide solution and heated to 90° C. until dissolution has taken place. The solution is cooled to 50° C., a solution of 4.5 parts of dimethylol urea in 5 parts of water is added and condensation for 13 hours is effected at temperatures between 50° and 60° C. Subsequently the solution is evaporated and a brownish powder results.

In the phenyl sulphones A to N the free sulphonic acid radicals are neutralized with concentrated sodium hydroxide solution and the solutions adjusted to a content of 5% in relation to the non-neutralized compounds. The phenyl sulphone O is neutralized with dilute sulphuric acid and the content brought to 5% based on the effective substance.

#### PHENYL SULPHONE P

3 parts of 100% sulphuric acid are added at room temperature to 25 parts of phenyl sulphone A (with an acid content as free acid of 340 mval./100 g.), heating is then effected to 140° and this temperature maintained for 1 hour. The mass is allowed to cool, neutralized with about 41 parts of 30% sodium hydroxide solution and evaporated to dryness. 40 parts of a light brown water soluble powder are obtained. The product has a similar formula to that of phenyl sulphone A, but at least one further H and in the Ph residue is replaced with  $-\text{SO}_3\text{H}$ .

Instead of the sodium hydroxide solution it is possible to use potassium or lithium hydroxide solution, sodium or potassium carbonate solution or even solid carbonates or bicarbonates of sodium, potassium or lithium. Furthermore, there may likewise be used as neutralization agent ammonia, magnesium oxide or carbonate, calcium oxide, hydroxide or carbonate, as well as solution of water soluble amines, for example methylamine, dimethylamine, trimethylamine, ethylamine, ethanolamine, diethanolamine, triethanolamine as well as the corresponding propanolamines and hexamethylenetetramine. Instead of sulphuric acid it is likewise possible to use other acids, for example hydrochloric acid, acetic acid, formic acid or even phosphoric acid as well as organic sulphonic acids (methane, benzene or 4-methylbenzene sulphonic acid).

The sulphones of the Formula A below, i.e. sulphones G to N above, are new; they are especially useful for dyeing barry-dyeing nylon and have the advantage of practically not foaming as do the known sulphonated

diphenyl oxides which contain a long aliphatic chain; furthermore, the compounds (A) are very good dispersing agents in acid or neutral medium and also, in contrast to e.g. sodium dinaphthylmethanedisulphonate, in alkaline medium.



(A)

10 wherein

m represents 1 or 2,

n represents 1, 2 or 3,

A<sub>1</sub> and A<sub>2</sub> are identical with or different from one another and each represents the residue of a compound of the formula

wherein X represents  $-\text{O}-$  or  $-\text{S}-$ , each of Z<sub>1</sub> and Z<sub>2</sub> represents a hydrogen atom or Z<sub>1</sub> together with Z<sub>2</sub> represents a single bond, and each of Z<sub>3</sub> and Z<sub>4</sub> represents hydrogen, halogen, lower alkyl or alkoxy, hydroxy, carboxy or optionally substituted phenyl, and each of p and q represents 1 or 2.

In the following examples, which illustrate the process of the invention, the parts are by weight, the percentages are by weight and the temperatures are stated in degrees centigrade. The quantities of phenyl sulphones stated in the examples relate to the condensation products with free  $-\text{SO}_3\text{H}$ -radicals in the case of phenyl sulphones A to N, or as the neutralized effective substance in the case of phenyl sulphone O.

#### EXAMPLE 1

40 A yarn consisting of 50 parts of nylon 6.6 and 50 parts of a spandex fibre Lycra [Ullmann 14351 (1963)] are dyed in 4000 parts of a dye bath containing the following ingredients: 0.25 part of sodium-1-amino-2-bromo-4-(4'-methyl-phenylamino)-anthraquinone - 2' - sulphonate (dyestuff I); 2 parts of 80% acetic acid; and 1.6 parts of phenyl sulphone A.

45 The yarn is put into the dye bath at 35° and heating to 95° is effected during 40 minutes. Dyeing at this temperature is effected for 1 hour. Both yarns are dyed level and in an even shade. When phenyl sulphone A is not added to the dye bath the dyestuff becomes preferentially adsorbed on the nylon 6.6 yarn and the Lycra yarn is dyed only in a pale shade.

50 An equally good result is obtained when the phenyl sulphone A is replaced with the same amount of one of the phenyl sulphones B, L or N.

#### EXAMPLE 2

55 50 parts of a nylon 6.6 yarn and 50 parts of a spandex fibre Lycra yarn are put in 3000 parts of a bath containing the following ingredients: 2 parts of 80% acetic acid; 2 parts of phenyl sulphone C. The yarn is put into the bath at 40° and the liquor is heated to 85° and kept at this temperature for 10 minutes. The bath is then cooled to 50° and 0.25 part of the dyestuff (I) are added. The bath is then heated during 10 minutes to 95° and dyeing at this temperature is effected for 1 hour. Both yarns are dyed level and in equal shade. When the phenyl sulphone C is not added to the dye bath the dye is preferentially adsorbed to the nylon 6.6 yarn and the Lycra yarn is dyed only in a pale shade.

60 Yarns likewise dyed level and in equal shade are obtained when 3 parts of phenyl sulphone E or 2 parts of one of the phenyl sulphones, G, H, K, M or O are used instead of the phenyl sulphone C.

## EXAMPLE 3

A yarn of 50 parts nylon 6.6 and 50 parts of spandex fibre Lycra are put into 4000 parts of a liquor containing the following ingredients: 3 parts of 80% acetic acid; 2.5 parts of phenyl sulphone A. The material is put into the bath at 40°, heating to 90° is effected and the liquor is kept for 20 minutes at this temperature. The bath is then cooled to 40° and 0.3 part of the sodium salt of 1-hydroxy-2-(3'-phenylaminosulphonyl-4'-methylphenylazo)-naphthalene-4-sulphonic acid (dyestuff II) are added. Subsequently heating to 95° is effected for 40 minutes and dyeing at this temperature is effected for 1 hour. The Lycra and the nylon 6.6 yarn are dyed in equal shade and level. When phenyl sulphone A is not added to the dye bath the dyestuff is mainly adsorbed on the nylon and the Lycra yarn is only dyed in a pale shade.

The 2.5 parts of phenyl sulphone A can be replaced without any difficulty with 2 parts of phenyl sulphone B or 3 parts of phenyl sulphone L.

When, instead of the dyestuff (II), there is used the same amount of a green dyestuff of the formula



green dyeings are produced which are similarly level and of equal shade.

## EXAMPLE 4

100 parts of the yarn mixture of Example 3 are treated in a solution of 2.5 parts of phenyl sulphone N and 2 parts of 80% acetic acid in 4000 parts of water for 15

5 minutes at 50°. 0.3 part of the dyestuff (II) are added to the bath and the liquor is heated for 40 minutes to 95° and kept for 1 hour at that temperature. The Lycra and nylon fibres are dyed in equal shade and level. When the phenyl sulphone N is not added to the dye bath the dyestuff is almost completely adsorbed to the nylon fibre, whereas the Lycra yarn is dyed only in a pale shade.

10 It is likewise possible to work with less dye liquor, e.g. 4000 or 5000 parts of water, without adversely affecting the results.

## EXAMPLE 6

15 Working is effected in the manner described in Example 5 with 8 parts of phenyl sulphone B in the pretreatment liquor and 0.3 parts of the dyestuff having the formula



20 are used. The Lycra yarn and the nylon yarn are dyed in an equal shade of blue, while without pretreatment the dyestuff is for the most part adsorbed in the nylon yarn and the Lycra yarn is only dyed in a pale shade.

## EXAMPLE 7

25 A yarn consisting of 50 parts of nylon 6 and 50 parts of a spandex fibre named Lycra are put into 4000 parts of a liquor containing the following ingredients: 2 parts of 80% acetic acid; 4 parts of phenyl sulphone A. The yarns are put into the liquor at 40°, heating to 90° is effected and this temperature is maintained for 15 minutes. The bath is then cooled to 40° and 0.25 part of a red dyestuff having the formula



30 minutes at 50°. 0.3 part of the dyestuff (II) are added to the bath and the liquor is heated for 40 minutes to 95° and kept for 1 hour at that temperature. The Lycra and nylon fibres are dyed in equal shade and level. When the phenyl sulphone A is not present in the dye liquor, the Lycra yarn is dyed in a substantially paler shade than the nylon 6 yarn.

## EXAMPLE 5

55

100 parts of the yarn mixture of Example 3 are pre-treated as in Example 3 with a solution of 2 parts of 80% acetic acid and 6 parts of the phenyl sulphone B in 6000 parts of water.

The bath is then cooled to 40° and 4 parts of ammonium sulphate and 0.25 part of the dyestuff of the formula



are added thereto. The dye bath is then heated during 45 minutes to 95° and kept for 2 hours at this temperature.

70 When the phenyl sulphone A is replaced with 3 parts of the phenyl sulphone B, very good results are likewise obtained.

75 A very good result is also obtained when the yarn mixture is first treated at 50° for 10 minutes in a solution of 4 parts of one of the phenyl sulphones A or L or 3

The Lycra and nylon yarn become level dyed in an equal shade of green.

One obtains likewise a dyeing of equal shade when the pretreatment of the yarn mixture is effected with 12 parts of the phenyl sulphone A and the actual dyeing is effected with 0.5 part of the dyestuff (IV). Without pretreatment the majority of the dyestuff is adsorbed on the nylon fibre and the Lycra fibre is only dyed in a pale shade.

It is likewise possible to work with less dye liquor, e.g. 4000 or 5000 parts of water, without adversely affecting the results.

## EXAMPLE 6

Working is effected in the manner described in Example 5 with 8 parts of phenyl sulphone B in the pretreatment liquor and 0.3 parts of the dyestuff having the formula



are used. The Lycra yarn and the nylon yarn are dyed in an equal shade of blue, while without pretreatment the dyestuff is for the most part adsorbed in the nylon yarn and the Lycra yarn is only dyed in a pale shade.

## EXAMPLE 7

A yarn consisting of 50 parts of nylon 6 and 50 parts of a spandex fibre named Lycra are put into 4000 parts of a liquor containing the following ingredients: 2 parts of 80% acetic acid; 4 parts of phenyl sulphone A. The yarns are put into the liquor at 40°, heating to 90° is effected and this temperature is maintained for 15 minutes. The bath is then cooled to 40° and 0.25 part of a red dyestuff having the formula



minutes at 50°. 0.3 part of the dyestuff (II) are added to the bath and the liquor is heated for 40 minutes to 95° and kept for 1 hour at that temperature. The Lycra and nylon fibres are dyed in equal shade and level. When the phenyl sulphone A is not present in the dye liquor, the Lycra yarn is dyed in a substantially paler shade than the nylon 6 yarn.

## EXAMPLE 8

100 parts of the yarn mixture of Example 3 are put at 40° into 10,000 parts of a dye liquor containing the following ingredients: 0.2 part of the 1:2-chromium complex compound of 1-(2'-hydroxy-5'-methylsulphonylphenylazo)-2-hydroxy-8-acetyl-amino - naphthalene (dyestuff (VII)); 4 parts of ammonium sulphate; 1 part of 80% acetic acid; and 3.6 parts of phenyl sulphone A.

The liquor is heated to 95° during 45 minutes and dyeing at this temperature is effected for 1 hour. The Lycra and nylon yarn are dyed in an equal shade of grey. When the phenyl sulphone A is not added to the bath, the dyestuff after the dyeing process is mainly adsorbed on the nylon yarn and the Lycra yarn is only dyed in a pale shade.

When the phenyl sulphone A is replaced with 3 parts of the phenyl sulphone B, very good results are likewise obtained.

A very good result is also obtained when the yarn mixture is first treated at 50° for 10 minutes in a solution of 4 parts of one of the phenyl sulphones A or L or 3

parts of the phenyl sulphone N or 6 parts of one of the phenyl sulphones C, F or K and 1 part of 80% acetic acid in 10,000 parts of water and then 4 parts of ammonium sulphate and 0.2 part of dyestuff (VII) are added, the dye liquor is brought to 95° in 45 minutes and dyeing is effected for 1½ hours at 95–100°.

Obviously the dyeing in a lesser amount of dye liquor, e.g. 6000 or 4000 parts of water, can be carried out with an equally good result.

This dyeing method is also very suitable for the dye-stuffs (IV), (V) or (VI).

#### EXAMPLE 9

100 parts of the yarn mixture of Example 3 are treated during 10 minutes at 50° in 4000 parts of a liquor which contains 1 part of ammonium sulphate and 6 parts of phenyl sulphone A. 0.1 part of the 1:2-chromium complex compound of 1-phenyl-3-methyl-4-(2-carboxy-phenylazo)-5-pyrazolone (dyestuff (VIII)) and 0.15 part of an anionic dispersing agent, e.g. sodium-di-naphthyl-methanedisulphonate or sodium-ligninsulphonate, are added. The dye bath is then heated to 95° during 45 minutes and this temperature is maintained for 1 hour. After the dyeing the Lycra and nylon yarns are dyed in an equal shade of yellow. When the phenyl sulphone A is not added to the dye bath, the dyestuff is mainly adsorbed on the nylon and the Lycra fibre is dyed only in a pale shade.

Instead of using 6 parts of phenyl sulphone A it is possible to use with equal success 2.5 parts of phenyl sulphone B or 4 parts of phenyl sulphone L or N, or 6 to 8 parts of phenyl sulphone F or the ammonium sulphate is replaced with 1 part of 80% acetic acid.

The dyestuff (VII) gives a level dyeing in an equal shade of grey.

#### EXAMPLE 10

100 parts of the yarn mixture of Example 3 are dyed in 4000 parts of a dye liquor containing the following ingredients: 0.25 part of the dyestuff of formula



4 parts of ammonium sulphate; 2 parts of 80% acetic acid; 1 part of one the phenyl sulphones G or H. The yarns are placed in the dye liquor at 40° and heating to 95° during 40 minutes is effected. Dyeing is effected at this temperature for 1 hour. Subsequently the liquor is cooled to about 70° and 3 parts of 85% formic acid and 1 part of potassium bichromate are added and heating is again effected to 95°. This temperature is maintained for 1 hour. The Lycra and nylon yarns are then dyed in an equal shade of yellow. When the phenyl sulphone A is not added to the dye liquor, the nylon 6.6 after dyeing has a deeper dye shade than the Lycra fibre.

Equally good results are obtained when the phenyl sulphone A is replaced with 1 part of the phenyl sulphones B, D, F or 1 part of a 1:1 mixture of phenyl sulphones A and F or 0.5 part of one of the phenyl sulphones A and N.

#### EXAMPLE 11

100 parts of yarn mixture of Example 3 are treated in a liquor of 4000 parts of water, 2 parts of 80% acetic acid and 3 parts of phenyl sulphone A at 80° during 15 minutes. The bath is then cooled to 40° and 0.25 part of the sodium salt of 1-hydroxy-2-phenylazo-6-(4'',6''-dichloro-1'',3'',5''-triazinyl-2''-amino) - naphthalene-3,2-disulphonic acid (dyestuff X) and 0.25 part of a phosphate buffer of pH value 7.0 are added to the liquor. The liquor is then heated to 95° and dyed at this temperature for 1½ hours. After the dyeing the Lycra yarn is clearly dyed. When the phenyl sulphone A is not present in the

dye liquor, the Lycra yarn is dyed in only a very pale shade.

Equally good results are obtained with one of the phenyl sulphones B and I.

#### EXAMPLE 12

A yarn consisting of 50 parts of nylon 6.6 and 50 parts of spandex fibre ESPA are treated at 80° for 10 minutes in 5000 parts of a liquor containing the following ingredients: 2 parts of 80% acetic acid; and 2 parts of phenyl sulphone A. The liquor is then cooled to 40° and 0.25 part of dyestuff (I) are added. The bath is then heated to 95° during 40 minutes and dyeing at this temperature is effected for 1½ hours. The ESPA and nylon yarns are dyed level and in an equal shade. When the phenyl sulphone A is not present in the dye bath, the dyestuff is almost completely adsorbed to the nylon yarn and the ESPA fibre is dyed only in a pale shade.

When the phenyl sulphone A is replaced with 2 parts of one of the phenyl sulphones B and N or 3 parts of the phenyl sulphone E or 3.5 parts of the phenyl sulphone F or 4 parts of the phenyl sulphone D, very good results are likewise obtained.

#### EXAMPLE 13

100 parts of a material consisting of 20 parts of spandex fibre Blue C and 80 parts of nylon 6.6 fibre are put into 400 parts of a liquor containing the following ingredients: 2 parts of 80% acetic acid; and 3 parts of one of the phenyl sulphones K, L or M.

The material is put into the liquor at 50° and this temperature is kept for 15 minutes. Subsequently 0.25 part of dyestuff (I) are added to the liquor and this is heated to 95° for 45 minutes. This temperature is maintained for 1 hour. A level dyed material results of equal colour shade. When no phenyl sulphone is added to the bath the Blue C fibres are practically undyed. For this reason the material has an unattractive aspect. This is particularly noticeable when the material is stretched.

Equally good results are obtained when 2.5 parts of phenyl sulphone A or 2 parts of phenyl sulphone B or 6 parts of one of the phenyl sulphones G and H are used.

#### EXAMPLE 14

A yarn consisting of 50 parts of nylon 6.6 and 50 parts of spandex fibre Rhodastic are dyed according to the dye method of Example 2, however, with the difference that the pretreatment is effected with 8 parts of one of the phenyl sulphones A and B and the dyeing itself with 0.5 part of dyestuff (I). After dyeing for 2 hours the Rhodastic fibre is dyed in a deep shade, whereas it is dyed only in a pale shade without any phenyl sulphone.

#### EXAMPLE 15

A yarn consisting of 50 parts of nylon 6.6 and 50 parts of spandex fibre "Bayer-Elastomer" is dyed according to the dye method of Example 2 using 1 part of phenyl sulphone A in the pretreatment bath. The nylon and spandex fibres are level dyed in an equal shade. When phenyl sulphone A is not present in the dye bath, the dyestuff is preferentially adsorbed on the nylon and the spandex fibre is dyed only in a pale shade.

Equally good results are obtained with 2 parts of one of the phenyl sulphones K and L. When the amount of phenyl sulphone A is increased to 6 parts and the dyestuff (I) is replaced with 0.5 part of dyestuff (VI), the spandex fibres are dyed in a noticeably deeper shade than the nylon, while in the absence of phenyl sulphone A the nylon is dyed in an appreciably deeper shade than the spandex fibres.

#### EXAMPLE 16

A yarn consisting of 50 parts of nylon 6 and 50 parts of a spandex fibre named Glospan is dyed according to the dye method of Example 2 using 1 part of one of the

